

March 18, 1924.

1,487,275

C. A. SCHARSCHU

ELECTROMETALLURGY

Filed Dec. 27, 1920

Fig. 1.



Fig. 2.



Inventor:  
Charles A. Scharschu,  
by *Albert G. Davis*  
His Attorney.

## UNITED STATES PATENT OFFICE.

CHARLES A. SCHARSCHU, OF PITTSFIELD, MASSACHUSETTS, ASSIGNOR TO GENERAL ELECTRIC COMPANY, A CORPORATION OF NEW YORK.

## ELECTROMETALLURGY.

Application filed December 27, 1920. Serial No. 433,147.

To all whom it may concern:

Be it known that I, CHARLES A. SCHARSCHU, a citizen of the United States, residing at Pittsfield, in the county of Berkshire, State of Massachusetts, have invented certain new and useful Improvements in Electrometallurgy, of which the following is a specification.

The present invention comprises a method 10 of and apparatus for refining steel and other metals and particularly silicon steel; the process results in a superior product which constitutes another aspect of my invention.

In the construction of cores for electrical 15 apparatus, especially of the alternating current type, such as transformers and dynamo-electric machines, it is highly important to use magnetic material in which the watt losses, due to hysteresis and eddy currents, 20 are as low as possible. Consequently efforts have been made during the development of the electrical industry to improve the magnetic properties of core material, and the substitution of silicon-iron and other alloys 25 for ordinary steel has indeed effected a considerable saving in electrical energy. Further efforts to still more improve the magnetic properties of silicon steel have and are being made by manufacturers of this 30 material, since it is realized that a reduction of core loss by even a small percentage results in the saving of a large amount of energy; thus a reduction of core loss of one or two per cent is looked upon as an 35 important achievement.

Silicon steel usually contains from 3.75% to 4% silicon; it is ordinarily made in the open hearth furnace; it is cast into ingots and these are rolled into thin sheets which 40 are used in core construction. The open hearth process results in a material in which a considerable amount of slag is distributed throughout the mass in which the sulphur content is generally as high as 45 from 0.03 to 0.04 per cent. I have found that the impurities carried by the slag and especially the high sulphur content of the product are detrimental characteristics of the magnetic material, since to their presence 50 a large percentage of the hysteresis action is due.

I have discovered that magnetic material of any kind and especially silicon steel may be made that is substantially free of slag in-

clusion and in which the sulphur content is 55 reduced to and below .010 and usually as low as 0.005 per cent, and even lower whereby the core loss is remarkably reduced, the reduction amounting on the average to about 12 per cent, and is in individual cases 60 still greater.

My improved process, broadly speaking, consists in treating the material, whether it be scrap or when already fused by the open hearth process, in a fluid state in such manner as to exclude the admission of air; expel the occluded particles of slag from the interior of the fused mass to the surface and then pour the material from underneath the sheet of slag which, as usually, is formed 70 on the surface. This process is preferably carried out by the use of an induction furnace of a specific construction which constitutes a part of my invention. While the fused mass is in the induction furnace and 75 preparatory to the practice of my invention, the material may be chemically refined in any ordinary or improved manner.

In the accompanying drawing, Fig. 1 illustrates partly in elevation and partly 80 in vertical section an induction furnace embodying structural features of my invention; Fig. 2 is a plan view of the furnace chamber, the furnace top being removed; and Fig. 3 is a top view, the primary coil 85 and housing being shown in part broken away.

The induction furnace shown in the drawing comprises an annular furnace crucible 1, surrounding a magnetic core 2, which has 90 a flat primary winding 3, supplied with alternating current by conductors not shown. The primary winding may consist of annular sections, as shown; it is suitably mounted on a framework 4 above the crucible 1, in the manner set forth in Patent No. 1326120 to Unger. The furnace crucible is provided with a refractory lining 5, which is in direct contact with the body of metal 6 to be melted, and consists preferably of particles of highly sintered or fused magnesia molded with a binder such as magnesium sulphate to form a solid mass. This lining rests upon a wall of refractory brick 7, which in turn is supported by a 100 suitable casing 8, made of boiler plate or the like. I have discovered that the location of the channel or crucible 1 beneath

the primary winding 3 subjects the molten mass in the crucible, constituting the secondary in the induction furnace, to the action of an alternating electromagnetic field 5 in such a manner that the slag particles occluded in the fused mass tend to separate from the metal, as will be hereinafter more fully explained.

The crucible 1 is provided with a refractory cover 9 which may consist of wedge-shaped sections, as shown in Fig. 3. The primary winding is preferably supported and surrounded by a shell 10 containing ventilating openings 11, but I wish it to 15 be understood that these and other structural details are shown merely for the purposes of illustration.

The pouring spout 12 communicates with the furnace chamber near the bottom like 20 the spout of a teapot, so that the fused metal may be poured from the furnace from beneath the top slag layer without causing this slag or any part of it to be mixed with the metal. The pouring spout is provided with 25 a door 13. The charge receiving opening 14 is similarly provided with a door (not shown). A pouring spout of this character has heretofore been suggested for use in another kind of furnace, but in the induction 30 furnace used for the practice of my process it cooperates with the magnetic function of the apparatus to assist the removal of the occluded slag particles.

The metal to be refined may be received 35 in a molten state from any suitable source, for example, a Bessemer converter, an open hearth furnace, or an arc furnace, and may consist of soft steel, hard steel, or any alloy steel. My invention is also applicable to 40 the melting of cold material either as scrap or new material directly in the induction furnace. The metal is allowed to attain a temperature of about 75° to 150° C. in excess of its melting point and is maintained 45 in that condition for a period of from 45 minutes to one and one-half hours in addition to the time required for chemical refinement if such is resorted to while the metal is in a fluid state in the induction 50 furnace.

When the induction furnace is charged with scrap or raw material, the ordinary chemical refinement is practiced right there, and after the refining slag has been removed 55 in the ordinary manner a new slag is added. This is preferably a basic slag consisting, for example, of lime and silica, the latter not exceeding 20%, and in some cases a small amount of fluorspar is added to thin 60 the slag. Any other suitable slag which is basic in character may be used. When chemically refined molten metal from any source, such as a Bessemer converter, an open hearth furnace or an arc furnace is introduced into the induction furnace, the 65

same procedure is observed, that is to say, a basic slag of the general character above indicated is added.

The molten metal is subjected to the electromagnetic purifying treatment which I 70 will now describe in greater detail. Owing to the location of the primary winding above the crucible element of the furnace, the alternating flux gives to the molten mass a slow but powerful movement from the inner edge of the annular channel downwardly toward the bottom and upwardly along the outer edge of the channel. In this respect the action of the flux upon the fluid metal is different from that of the magnetic 80 flux when the primary winding is concentric with the channel, for in the latter case the molten metal is violently agitated in an irregular manner, causing the occluded slag particles to mix continuously with the metal 85 and effectually preventing a separation of the same. By locating the primary winding above the crucible channel, the movement of the metal becomes very much slower. There are two forces acting on the molten charge 90 tending to expel the slag from the metal, namely, the compressive effect of the magnetic field upon the charge and the electrodynamic effect which exerts a different repellent action upon the slag and metal. 95

The compressive or pinch force of the magnetic field of a current-carrying conductor is a force acting radially inward upon the current-carrying elements of the conductor. As the slag is a poor conductor it tends 100 to be squeezed out somewhat like water being squeezed out of a sponge. The separating action due to the electro-dynamic effect is somewhat comparable to the separation occurring in a centrifugal separator. The 105 current-carrying metal is repelled with greater force than the slag particles. As the magnetic field is applied from above, the slag particles tend to come to the surface. Due to the combined effect of the slow and regular movement of the charge and the expulsive force exerted on the slag particles, they are carried with the metal to the surface and there attach themselves to the slag. In this manner the fused mass is substantially freed from slag occlusion. 115

My improved form of pouring spout 12 which communicates with the bottom of the crucible 1 prevents the remixing of the metal with the expelled slag when the metal is 120 poured by tilting the furnace, so that the advantage of the preceding melting treatment under the influence of the electromagnetic field is not lost when the metal is poured.

What I claim as new and desire to secure by Letters Patent of the United States, is:—

1. The method of refining metal containing slag particles which consists in subjecting said metal in a molten state to a period- 120

ically varying magnetic field adapted to cause said slag particles to rise to and remain on the surface and thereupon separating the metal and slag while preventing 5 re-admixture thereof.

2. The steps in the method of refining metal which consists in subjecting said metal in a molten state to the effect of a periodically varying magnetic field applied from 10 above the body of metal to be purified, thereby causing slag inclusions to rise to and remain at the surface, and finally separating the purified metal from the superimposed slag layer while said layer remains undisturbed.

3. The steps in the method of refining alloys which consists in subjecting said alloys at a temperature materially in excess of the melting point, subsequent to purification by chemically active reagents, to a 20 periodically varying magnetic field acting to separate slag particles from said alloy and

then casting said alloy while preventing remixture of said alloy and slag.

4. The method of refining silicon steel 25 which consists in subjecting said steel at a temperature above the melting point in contact with a slag to a periodically varying magnetic field applied from above said steel, thereby causing impurities in said steel 30 to be incorporated into the slag and finally separating the metal and slag while maintaining said slag undisturbed.

5. The method of refining ferrous metal 35 which consists in electromagnetically expelling slag particles from said metal while in a molten state and thereupon mechanically separating said metal from supernatent slag while preventing readmixture between metal and slag.

In witness whereof, I have hereunto set my hand this 22nd day of December, 1920.

CHARLES A. SCHARSCHU.